

June 10, 1930.

O. GLOESER

**1,762,815**

## MANUFACTURE OF REINFORCED CONCRETE

Filed April 26, 1928



Fig.2



Fig.4



Fig. 5



*Inventor:*

Ott. Glessner

## UNITED STATES PATENT OFFICE

OTTO GLOESER, OF NIKLASDORF, NEAR FREIWALDAU, CZECHOSLOVAKIA

## MANUFACTURE OF REINFORCED CONCRETE

Application filed April 26, 1928, Serial No. 273,020, and in Germany April 28, 1927.

The present invention relates to a process of producing solid and hollow reenforced concrete constructions such as concrete poles and the like, and has for its object to prevent as much as possible fine cracks in the concrete, which soon damage the latter and render the construction useless.

These hairline cracks, which develop in a very troublesome manner in the existing type 10 of reenforced concrete constructions, are prevented, according to the present invention, by tensioning reenforcement bars up to their elastic limit before the concrete is rammed and by compressing the still liquid concrete 15 by means of a press plate guided by the reenforcement bars until it hardens so that the hardened concrete remains under the constant pressure of the bars when the tension device is released.

20 One form of the invention is illustrated in the accompanying drawing of a pole, in which Figure 1 is a view of the reenforcement bars under tension; Fig. 2, a perspective view of the lower tension plate; Fig. 3, a view of the 25 finished pole; Fig. 4, a section on the line A—B Fig. 3; and Fig. 5, a cross section of the pressing mold of the pole with inserted core.

Referring to the drawing, 1 is the head 30 plate into which any number, for instance 6, of reenforcement bars 2 are screwed. The free ends of the bars 2 pass through a press plate 3 adapted to be shifted on the bars 2 in the direction of the arrow I by means of 35 the nuts 4. The ends of the reenforcement bars are attached by the nuts 5 to the tension plate 6 provided with the hooks 7 which engage the eyelets 9 arranged in a wall 8 or the like. The head plate 1 is fitted with an 40 eyelet 10 hooked up with a tensioning device 11 comprising a sort of tackle which in turn has a hook adapted to engage the eyelet 12 arranged in a wall or the like. Both the tension plate 6 and the press plate 3 have 45 a central aperture 13 through which a core 14 (Fig. 5) can be inserted to obtain a hollow pole.

The process of producing reenforced concrete constructions according to this invention 50 consists in tensioning the reenforcement

bars 2 up to their elastic limit by means of the tightening device 11, inserting the core 14 through the apertures 13 of the press and tension plates 3 and 6, and in arranging in the core 14 the radial projections 15 for the 55 purpose of providing the requisite climbing openings 16, whereupon the reenforcement bars are covered helically with the wire 17.

Over and around the tensioned reenforcement bars 2, which have been provided with 60 the cores 14 and 15, the mold 18 is arranged so that liquid concrete can be successively rammed into it, whereupon it is gradually being closed and its parts are tightened by means of the screws 19. As soon as this has 65 been done, the nuts 4 of the press plate 3 are tightened as far as possible so that the press plate 3 can be shifted on the reenforcement bars 2 in the direction of arrow I to compress the still liquid concrete mass 20, 70 the water contained in the latter escaping through the mold 18 or on the two face sides, so that the concrete becomes very dense and is free from porosity.

After the concrete mass 20 has hardened 75 completely the nuts 4 of the tension plate 3 are tightened as much as possible while the tightening device 11 is relieved. The reenforcement bars 2 are thus enclosed in tensioned condition in the concrete, and the tensile stress still present in them is absorbed 80 or taken up by the set concrete as compressive stress.

Aside from poles all other kinds of reenforced concrete constructions can be produced in this manner and will be superior 85 to the prevailing types employing untensioned reinforcements in so far as they will show much greater strength at lower weight. 90

The number of reenforcement means used as well as the shape and cross section of the constructions can be altered to suit requirements without affecting the invention.

I claim:—

The process of reenforcing concrete consisting in forming a body of concrete with the reenforcement embedded therein, in tensioning the reenforcement up to its elastic limit before the concrete is rammed, in com- 100

pressing the still liquid concrete by suitable apertured means guided by the reenforcement, and finally in releasing the tensioning means after the concrete has set.

5 In testimony whereof I have affixed my signature.

OTTO GLOESER.

10

15

20

25

30

35

40

45

50

55

60

65